

## UNITED STATES PATENT OFFICE.

RUDOLF SAJITZ AND FRIEDRICH POSPIECH, OF DRESDEN, GERMANY, ASSIGNEES TO CHEMISCHE FABRIK POTT & CO., OF DRESDEN-N., GERMANY.

## METHOD OF SPINNING ARTIFICIAL FILAMENTS.

No Drawing. Application filed June 14, 1926, Serial No. 116,012, and in Germany June 17, 1925.

This invention refers to a process of facilitating the manipulation and improving the spinning qualities of cellulose-solutions, viscose and the like. In the manufacture of artificial silk from cellulose solutions there are sometimes difficulties in the formation of the threads, inasmuch as, when the two heterogeneous systems of material, the spinning solution and the precipitating bath are made to act upon each other, surface tension is produced which has an unfavorable influence upon the formation of the threads.

Now, we have ascertained that these difficulties may be overcome with certainty, if provision is made to reduce the surface tension on the bounding surfaces of the two systems by the addition of suitable substances. As substances to be added for this purpose we have found according to our invention small amounts of naphthalene-sulphonic acid which are alkyl-substituted in the ring, or their salts or other derivatives to be particularly suitable, and of these naphthalene-sulphonic acids have been shown to be preferable which are substituted by alkyls with several carbon-atoms, and the salts and derivatives of such sulphonic acid. We have found that such sulphonic acids of naphthalene are very well suitable for the purpose which, besides the substituting alkyl-groups contain a plurality of sulpho-groups in the core, and of these particularly the di- and tri-sulphonic acids may be used with preference, and as such for instance isopropyl-naphthalene-di-sulphonic acid. The particular important advantage of the employment of this kind of sulphonic acids for the purpose in question resides in the fact that they possess an almost unlimited solubility.

It is only necessary to add a small quantity of these substances either to the cellulose-solutions themselves or to the precipitating baths employed in each case, or to both of them at a time. By the employment of these substances the spinning process is facilitated and on the other hand the quality of the threads themselves is very favorably influenced.

The process may be employed with cellulose-solutions of all kinds, such as solutions in copper-oxide-ammonia, chloride of zinc,

and for cellulose-acetate solutions, viscose-solutions and similar solutions.

## Examples for the carrying out of the process. 55

1. 10 kilogrms. of a cellulose-acetate spinning solution are treated with a solution of 10 grms. of the purified sodium-salt of the substituted beta-naphthalene-sulphonic acid 60 in the just sufficient quantity of acetone or acetic-ester, such as may be obtained by a suitable condensation of beta-naphthalene-sulphonic acid with the mixture of higher alcohols which are obtained in the hydrogenation of the subsequent distillation residues of acetone.

2. To each 10 kilogr. of a precipitating solution comprising dilute sulphuric acid saturated with sodium-sulphate 100 grms. of 70 isopropyl-naphthalene-sulphonic acid are added, such as may be obtained by a suitable condensation of beta-naphthalene-sulphonic acid with isopropyl-alcohol, and the usual purification.

3. To each 100 kilogr. of a precipitating bath which consists of dilute sulphuric acid, saturated with sodium-sulphate 100 grms. iso-propyl-naphthalene-di-sulphonic acid are added, such as may be obtained by a suitable 80 condensation of beta-naphthalene-sulphonic acid with isopropyl-alcohol and suitable purification.

It will, of course, be understood that the invention is not restricted for its execution 85 to the particular kinds of material and proportions hereinbefore recited for the purpose of exemplification, but it is susceptible of changes and modifications in the selection of such substances and of their relative proportions without deviating from the spirit and scope of the invention, as particularly pointed out in the appended claims.

## We claim:—

1. The process of improving the spinning 95 qualities of cellulose-solutions, which consists in treating such solutions with precipitating agents in the presence of naphthalene-sulphonic compounds, containing substituted alkyl-radicals and several sulpho-substitution groups in the ring.

2. The process of improving the spinning qualities of cellulose-solutions of all kinds, which consists in treating such solutions

with precipitating agents in the presence of naphthalene-sulpho-compounds, containing iso-propyl radicals in the ring.

3. The process of improving the spinning qualities of cellulose-solutions, which consists in precipitating the same in the presence of ring-alkaly-substituted naphthalene-poly-sulphonic acids.

4. The process of improving the spinning

qualities of cellulose-solutions of all kinds <sup>10</sup> which consists in precipitating the same with sulphuric acid-baths, containing alkali-sulphates and in the presence of iso-propyl-ring substituted naphthalene-sulphonic acid compounds.

**RUDOLF SAJITZ**  
**FRIEDRICH POSPIECH.**